

[54] INK RIBBON HAVING AN ANISOTROPIC ELECTRIC CONDUCTIVITY

[75] Inventors: **Jacques Ehretsmann**, Conches/Geneve; **Emile Barbey**, Geneve; **Paul Heinzer**, Zurich, all of Switzerland

[73] Assignee: **Battelle Memorial Institute**, Carouge/Geneva, Switzerland

[22] Filed: **Apr. 25, 1973**

[21] Appl. No.: **354,181**

[30] Foreign Application Priority Data

Apr. 26, 1972 Switzerland ..... 6235/72

[52] U.S. Cl. .... **197/172**, **117/238**, **346/76 R**

[51] Int. Cl. .... **B41j 31/02**

[58] Field of Search ..... **197/172**, **1 R**; **101/467**, **101/468**, **469**, **470**; **117/217**, **218**, **235**, **238**; **346/76 R**

[56] References Cited

UNITED STATES PATENTS

2,796,359 6/1957 Speed ..... 117/238

|           |         |                     |             |
|-----------|---------|---------------------|-------------|
| 2,917,996 | 12/1959 | Epstein et al. .... | 346/76 R UX |
| 3,001,891 | 9/1961  | Stoller.....        | 117/238     |
| 3,117,065 | 1/1964  | Wootton .....       | 117/238     |
| 3,318,697 | 5/1967  | Shrewsbury.....     | 101/469 UX  |
| 3,441,940 | 4/1969  | Salaman et al. .... | 346/76 R X  |
| 3,570,380 | 3/1971  | Kamenstein.....     | 197/1 R UX  |
| 3,588,912 | 6/1971  | Hackett.....        | 346/76 R    |
| 3,599,228 | 8/1971  | Coco et al. ....    | 346/76 R    |

OTHER PUBLICATIONS

IBM Technical Disclosure Bulletin, "Magnetic Transfer Medium," Miller et al., Vol. 7, No. 6, November 1964, page 422.

Primary Examiner—Ernest T. Wright, Jr.

Attorney, Agent, or Firm—Hubbell, Cohen & Stiefel

[57]

ABSTRACT

Polymeric ribbon having a plurality of chains of magnetized ferromagnetic conductive particles extending through the ribbon to yield an ink ribbon having an anisotropic electrical conductivity extending in the direction of the thickness of the ribbon.

6 Claims, 4 Drawing Figures



PATENTED NOV 12 1974

3,847,265



FIG. 1



FIG. 2



FIG. 3



FIG. 4

## INK RIBBON HAVING AN ANISOTROPIC ELECTRIC CONDUCTIVITY

This invention relates to an ink ribbon having anisotropic electric conductivity.

French Pat. No. 2,069,525 describes a printing mechanism provided with an ink ribbon formed by a flexible support having an electric conductivity which is greater in the direction of its thickness than in the plane of its major surfaces, one surface of the support being coated with an ink which is both thermofusible and electrically conducting.

The difference in conductivity of this ribbon is essentially due to the provision of a plurality of conductive elements in the mass of the ribbon, the conductive elements extending from one side to the other through the thickness of the ribbon.

With this ribbon the printing operation proper is effected by locally pressing the inked surface of the ribbon against the surface to be printed and each time connecting one or more pairs of conductive elements to a first and a second terminal of a source of current for the first element and the second element of each pair, respectively, so that electric current is fed through the portion of the ink layer between the two elements of each pair and consequently this portion of the ink layer is melted by the Joule effect thus produced.

Such a ribbon has however some disadvantages both with respect to its production and its use. Among the disadvantages in use are the very stylized form of the obtained characters, the very limited number of possibilities in the choice of the lines produced with a group of given letters, and the difficulty of selecting the electrodes from a group of electrodes occupying a very small surface on the ribbon.

Therefore, it has been proposed in this French Patent to use a ribbon having an anisotropic electric conductivity in the direction of its thickness.

It is therefore an object of the present invention to provide an ink ribbon having an anisotropic electric conductivity in the direction of its thickness and which is characterized in that it is formed of a resin containing a plurality of chains of electrically conductive particles extending through the ribbon in the direction of its thickness.

The accompanying drawing shows, schematically and merely by way of example, a preferred embodiment of means for producing the ribbon of the present invention according to different processes. In the drawing;

FIG. 1 is an elevational view of the ribbon producing means;

FIG. 2 is a sectional view taken on the line II-II of FIG. 1;

FIG. 3 is a transverse sectional view, taken on an enlarged scale, through a mould for producing the ribbon; and

FIG. 4 is a perspective view, on an enlarged scale, of a piece of ribbon obtained by the process of the present invention.

In a first form of carrying out the process for producing the ink ribbon, first nickel powder is mixed with a prepolymer, for example, Rhodester (Trade-Mark of Rhone-Poulenc), and then a surfactant, which also serves as a dispersing agent, in the present case magnesium stearate, is added to the mixture in a proportion of 0.2 percent.

The prepolymer may be a Rhodester 1103 or a mixture of Rhodester 1103 and 1108. Rhodester 1103 is a prepolymer of polyester containing 45 percent of styrene. Its density at 25°C. is 1.06 before polymerization and 1.18 after polymerization. Its acid and hydroxyl values are both 10. Rhodester 1108 is a prepolymer of polyester containing 30 percent of styrene. Its density at 25°C. is 1.14 before polymerization and 1.23 after polymerization. Its acid value is 34 and its hydroxyl value is 42.

To prepare the mixture of nickel powder and Rhodester 1103 or the mixture of nickel powder and Rhodester 1103 and 1108, the nickel powder and the surfactant are dispersed in the prepolymer by subjecting the mixture to vibrations of a supersonic frequency. Then a catalyst is added to the mixture in a ratio of 0.3 percent to produce polymerization and an accelerator is added in a ratio of 0.1 percent to accelerate the reaction.

This mixture is then spread in the form of a layer 1 on a thin glass plate 2, as shown in FIG. 3. Previously spacer blocks 3 having a thickness of between 0.2 and 0.6 mm, depending on the thickness of the ribbon to be produced, are placed on the glass plate 2. Then a second glass plate 4 similar to the first one is placed on the blocks 3 to form a sandwich structure which is inserted in the air gap 5 of an electromagnet 6 formed by a coil 7 placed in a soft iron armature 8 having the form of an E in cross section. A cover 9 likewise of soft iron is placed on the armature 8, the cover 9 being provided with a longitudinal rib 9a facing the central rib 8a of the armature 8. The air gap 5 is located between the ribs 8a and 9a and has an elongate form, its dimensions being such that the aforementioned sandwich structure can be inserted therein.

After the sandwich structure has been placed into the air gap 5 the coil 7 is energized to produce a magnetic field in the air gap 5 so that the lines of force of the magnetic field traverse the sandwich structure. The magnetic field traversing the mixture 1 which is still in the liquid state produces an alignment of the nickel particles contained in the mixture 1 in the form of chains extending transversely in the direction of the thickness of the ribbon, i.e., along the lines of force of the magnetic field.

After this first form of carrying out the process of producing an anisotropic ink ribbon has thus been described, let's examine the influence of certain parameters on the anisotropic ribbons produced by means of the apparatus which so far has been summarily described. The results of these parameters and particularly the resistivity of the ribbon in its transverse direction are indicated in the following Table I.

TABLE I

| Sample No. | Nickel Type | % by weight | Ribbon thickness ( $\mu$ ) | Magnetic Oe | field duration in hrs. | Transverse resistivity Ohm/cm <sup>2</sup> |
|------------|-------------|-------------|----------------------------|-------------|------------------------|--------------------------------------------|
| 22         | B 20 - 40   | 20          | 100-200                    | 2700        | 2.5                    | 6                                          |
| 40a        | T 255       | 20          | 110-120                    | 5800        | 1                      | 0.8                                        |
| 40b        | B20 - 40    | 30          | 80-90                      | 3350        | 1                      | 0.3                                        |
|            | SF 300      | 34          |                            |             |                        |                                            |

3  
TABLE I—Continued

| Sample No. | Nickel Type | % by weight | Ribbon thickness ( $\mu$ ) | Magnetic field Oe | duration in hrs. | Transverse resistivity Ohm/cm |
|------------|-------------|-------------|----------------------------|-------------------|------------------|-------------------------------|
| 42a        | SF 300      | 50          | 100-120                    | 5800              | 1                | 0.36                          |
|            | OSF 10      | 10          |                            |                   |                  |                               |
|            | OSF 5       | 10          |                            |                   |                  |                               |
| 42b        |             |             | 90-100                     | 3350              | 1                | 0.4                           |
| 44a        | B 20-40     | 50          |                            | 5800              | 1                |                               |
| 44b        | SF 300      | 60          | 110-120                    | 3350              | 1                | 0.36                          |
| 45a        | B 20-40     | 50          | 110-120                    | 2700              | 1                | 0.36                          |
| 45b        | SF 300      | 60          | 100-110                    | 1000              | 1                | 0.6                           |

The origin and dimensions of the nickel powders mentioned in this table are indicated in the following Table II.

| Type    | Diameter ( $\mu$ ) | Manufacturer                      |
|---------|--------------------|-----------------------------------|
| OSF 5   | 5                  | Sheritt Gordon Mines Ltd., Canada |
| OSF 10  | 10                 |                                   |
| SF 300  | <50                | Mond Nickel Co.                   |
| T 255   | 2                  |                                   |
| B 20-40 | 20-40              | Baudier, France                   |

The values of transverse resistivity given in ohm/cm in Table I are obtained by placing an electrode on each side of the ribbon and exerting a slight pressure on each of the electrodes and connecting the latter, for example, to an ohmmeter.

In all the samples indicated in Table I the coefficient of anisotropy given by the ratio between the resistance measured in a direction parallel to the surface of the ribbon and the resistance measured in a direction perpendicular to this surface is higher than 10<sup>6</sup> and thus excellent.

As will be seen by referring to Table I, some of the indicated samples contain nickel powders of different origin and particle size which are indicated in Table II.

It has been found that this mixture of particles generally results in an improvement of the conductivity in the transverse direction of the ribbon, particularly when the medium diameter of the particles is different. It has also been found that the presence of large particles tends to produce a reduction in the resistivity of the ribbon. Further, by increasing the concentration of the nickel powder ribbons of better characteristics and the same good coefficients of anisotropy have been obtained.

The orientation of the nickel particles by the magnetic field during the production of the ribbon takes place rather rapidly, namely in the first 5 to 10 minutes. This is because after this period the polymerization initiated by the catalyst imparts to the prepolymer used as the starting material a viscosity which is so high that the nickel particles can no longer move under the influence of the lines of force of the magnetic field traversing the ribbon.

To form the insulating portion of the ribbon practically any type of plastics material may be used such as heat-setting monomers, prepolymers, copolymers or polymers which initially are in the form of a liquid having a sufficiently low viscosity to permit the orientation of the nickel particles under the influence of the magnetic field. The polymer obtained after polymerization

must have certain plastic properties such as sufficient flexibility but low elasticity.

To prepare the sample of the ribbon No. 22 of the Table I, a mixture of two prepolymers, the aforementioned Rhodester 1103 and 1108, has been used in the ratio of 7 to 3. For the samples of the ribbons No. 40 to 45 only Rhodester 1103 has been used. The mechanical properties of the polymer thus obtained are not as good as those of the polymer obtained by the mixture of Rhodester 1103 and 1108 but the polymer made of Rhodester 1103 only has better properties of contact when an electrode is applied to the surface of the ribbon.

According to a second form of carrying out the process of producing an anisotropic ink ribbon, a thermoplastic or fusible resin is used which is heated to its melting point and then nickel powder is added to this resin by mixing it while the resin is in the molten state. Then this mixture is placed into a mould of the type shown in FIG. 3, taking care that this mould has been heated previously to a temperature corresponding to that of the melting point of the thermoplastic material employed, and then the mould is placed into the air gap 5 of the electromagnet 6 which is then energized to produce an orientation of the metal particles of the mixture while the mixture is cooling and hardening as was described with reference to the first form of carrying out the process.

According to a modification of this form of carrying out the process and if the speed of hardening of the resin is too high, small resistances may be arranged to extend through the mould to keep the latter at a certain temperature and control the speed of lowering of the temperature of the mixture.

Obviously this second form of carrying out the process may also be applied to a thermo-setting resin with which nickel powder would be mixed. Then this mixture is placed into a mould such as that shown in FIG. 3, the mould is placed into the air gap 5 of the electromagnet 6 which is energized and simultaneously the mould is heated, for example, by means of electric resistances (not shown) extending through the mould, to harden the resin.

FIG. 4 shows a piece of the ribbon 1 obtained by the process described above and having an anisotropic electric conductivity. On the surface of this ribbon there can be seen the metal particles P to which an electrode can be applied and chains of particles C<sub>1</sub>, C<sub>2</sub>, . . . C<sub>n</sub> appear on the side 1b of the ribbon and form electrically conductive passages between the two surfaces 1a and 1c of the ribbon.

We claim:

1. An ink ribbon having an anisotropic electric conductivity in the direction of the thickness of the ribbon, characterized in that said ribbon is formed of a resin containing a plurality of chains of electrically conductive particles extending through the ribbon in the direction of said thickness.

2. An ink ribbon as claimed in claim 1, characterized in that said electrically conductive particles comprise a ferromagnetic metal.

3. An ink ribbon as claimed in claim 1, characterized

in that said electrically conductive particles have a diameter between 2 and 50 $\mu$ .

4. An ink ribbon as claimed in claim 1, characterized in that said resin is a polyester polymer.

5. An ink ribbon as claimed in claim 1, characterized in that said resin is a thermo-setting resin.

6. An ink ribbon as claimed in claim 1, characterized in that said resin is a thermoplastic resin.

\* \* \* \* \*

15

20

25

30

35

40

45

50

55

60

65

**Dedication**

3,847,265.—*Jacques Ehretsmann, Conches/Geneve; Emile Barbey, Geneve and Paul Heinzer, Zurich, Switzerland. INK RIBBON HAVING AN ANISOTROPIC ELECTRIC CONDUCTIVITY.* Patent dated Nov. 12, 1974. Dedication filed Mar. 26, 1984, by the assignee, *Battelle Memorial Institute.*

Hereby dedicates to the People of the United States the entire remaining term of said patent.

[*Official Gazette May 29, 1984.*]